

1

2,780,597

## LUBRICATING COMPOSITIONS

Paul H. Williams, Berkeley, Lawrence B. Scott, Lafayette, and Victor N. Borsoff, Berkeley, Calif., assignors to Shell Development Company, Emeryville, Calif., a corporation of Delaware

No Drawing. Application July 18, 1952,  
Serial No. 299,741

12 Claims. (Cl. 252—18)

This invention relates to lubricants particularly suitable for lubrication under extreme operating conditions, such as under extreme pressure, high speed and high temperature conditions.

It is well known that the high pressure occurring in certain types of gears and bearings may cause a film of lubricant to rupture with consequent damage to the machinery. It has been shown that base lubricants such as mineral oil and/or synthetic oil can be improved with regard to their protective effect particularly on rubbing surfaces by the addition of certain substances, so that excessive wear, scuffing and seizure, which normally follow a break in the film of lubricant, can be prevented even under very unfavorable pressure and speed conditions. Lubricants possessing this highly desirable property are called extreme pressure lubricants.

It is known that certain elements or compounds of elements of the type of chlorine, sulfur, phosphorus and lead are capable of imparting extreme pressure properties to lubricants, which may be lubricating oils and greases, when blended therewith. Among the compounds heretofore used are notable the lead soaps, phosphoric acid esters, free sulfur, and certain chlorinated organic compounds. A principal objection to extreme pressure compounds of this class is that they are highly reactive with contacting surfaces causing etching, corrosion and discoloration of said surfaces. Another objection to reactive extreme pressure agents is that they alter the original chemical nature of the contacting surface and this, under certain conditions, is undesirable. Additionally, because of the activity of agents of the type under discussion they usually deplete rapidly resulting in, at the very best, only a temporary solution to extreme pressure lubrication.

It has now been discovered that improved extreme pressure lubricants can be obtained by incorporating into a base lubricant, minor amounts of certain inorganic salts in the form of colloidal particles, of from less than 1 to 10 microns and preferably from less than 0.5 to 3 microns, said colloidal salts being capable of forming under conditions of use viscous liquids or glass-like solids which have a greater affinity for contacting surfaces to be lubricated than the base lubricant or liquid carrier.

The colloidal inorganic salts include metal and/or ammonium acid phosphates, silicates, antimonates, molybdates and mixtures thereof. Specific examples of compounds which are particularly suited in compositions of this invention include: sodium, potassium and ammonium mono and dihydrogen phosphates, acid silicates and mixtures thereof.

Salts and their mixtures of this invention which might lack desired oil solubility can be sufficiently oil solubilized in desirable base carriers by mechanical means such as described in U. S. Patent 2,529,461 or by grinding in colloidal or paint mills or any other suitable means. Still another method of maintaining the salts of this invention in bases such as oils is by means of dispersing agents.

2

In selecting suitable dispersing agents, they must be of such a nature as to be oil soluble, have good dispersing properties, but possess less of an affinity or attractiveness for the surface to be lubricated than the salts of this invention. Dispersing agents which are practically preferred

5 include esters of polyhydric alcohols and derivatives thereof, such as propylene glycol monolaurate, propyl glycol mono-oleate, propylene glycol monostearate, oleic acid derivative of polyoxyethylene sorbitol (G-1096, Atlas Powder Co.), polyoxyalkylene glucose tetrastearate (G-1164, Atlas Powder Co.), glycerol sorbitan laurate (G-672, Atlas Powder Co.), and the like.

10 Salts of this invention are excellent activating or "spiking agents" for well known extreme pressure agents such as organic phosphates, phosphonates, sulfur containing compounds, chlorine containing compounds and mixtures thereof. By "spiking agents" is meant materials capable of activating and improving the load carrying and extreme pressure properties of the general class of compound enumerated above, and particularly such compounds as the full and partial esters of trichloromethane-phosphonic acid and their salts (monobutyl trichloromethane phosphonate, di-2-ethylhexylamine salt of monobutyl trichloromethane phosphonate), sulfurized and/or phosphorized fatty oils and waxes, chlorinated waxes and the like.

15 Base oils to which agents of this invention are added may be selected from a variety of natural oils such as paraffinic, naphthenic, and mixed base mineral oils having 20 a viscosity range such as from 40 at 100° F., SUS, to up to 1000 SUS at 210° F. In addition, synthetic oils may be used such as polymerized olefins, alkylated aromatics; polyalkyl silicone polymers, e. g., liquid dimethyl silicone polymer, other silicone polymers; H<sub>2</sub>S-adducts 25 of unsaturated ethers and thioethers, e. g., H<sub>2</sub>S adduct of diallyl ether; esters, e. g., di(2-ethylhexyl) sebacate. Mixtures of natural and synthetic oils can be used. Under certain conditions of lubrication, minor amounts of a fixed oil such as castor oil, lard oil and the like, may 30 be admixed with a hydrocarbon oil and/or synthetic oil.

35 The general formulation of compositions of this invention can be represented by:

| 45 | Extreme Pressure Agent(s)                                                                                                | Amount (Percent by wt.) |                 |
|----|--------------------------------------------------------------------------------------------------------------------------|-------------------------|-----------------|
|    |                                                                                                                          | Broad Range             | Preferred Range |
| 50 | Certain inorganic salts, e. g., KH <sub>2</sub> PO <sub>4</sub> , (NH <sub>4</sub> ) <sub>2</sub> PO <sub>4</sub> , etc. | 0.01-10<br>1-20         | 0.1-5<br>1-10   |
|    | Dispersing (optional): Preferred ester type.                                                                             |                         |                 |
|    | Optional Additive: Organic extreme pressure agents, detergents, anti-oxidants, corrosion inhibitors, etc.                | 0.01-5                  | 0.1-2           |

55 Preferred compositions of this invention are illustrated by the following examples:

### Composition A

KH<sub>2</sub>PO<sub>4</sub> percent 2  
Mineral oil Balance

### Composition B

NaH<sub>2</sub>PO<sub>4</sub> percent 2  
Mineral oil Balance

### Composition C

(NH<sub>4</sub>)<sub>2</sub>PO<sub>4</sub> percent 2  
Mineral oil Balance

### Composition D

KH<sub>2</sub>PO<sub>4</sub> percent 2  
Glycerol sorbitan laurate (G-672, Atlas Powder Co.) percent 6  
Mineral oil Balance

## Composition E

|                                  |         |   |
|----------------------------------|---------|---|
| NaH <sub>2</sub> PO <sub>4</sub> | percent | 2 |
| Glycerol sorbitan laurate        | do      | 6 |
| Mineral oil                      | Balance |   |

## Composition F

|                                                                                  |         |   |
|----------------------------------------------------------------------------------|---------|---|
| KH <sub>2</sub> PO <sub>4</sub> + H <sub>3</sub> BO <sub>3</sub> (50-50 mixture) | percent | 2 |
| Glycerol sorbitan laurate                                                        | do      | 6 |
| Mineral oil                                                                      | Balance |   |

## Composition G

|                                                                      |         |   |
|----------------------------------------------------------------------|---------|---|
| KH <sub>2</sub> PO <sub>4</sub>                                      | percent | 2 |
| Di-2-ethylhexyl amine salt of monobutyl trichloromethane phosphonate | percent | 1 |
| Mineral oil                                                          | Balance |   |

## Composition H

|                                                                      |         |   |
|----------------------------------------------------------------------|---------|---|
| (NH <sub>4</sub> ) <sub>2</sub> PO <sub>4</sub>                      | percent | 2 |
| Di-2-ethylhexyl amine salt of monobutyl trichloromethane phosphonate | percent | 1 |
| Mineral oil                                                          | Balance |   |

## Composition I

|                                                                         |         |   |
|-------------------------------------------------------------------------|---------|---|
| KH <sub>2</sub> PO <sub>4</sub>                                         | percent | 2 |
| Ucon Fluid (polyether compound sold by Carbide and Carbon Chemical Co.) | Balance |   |

## Composition K

|                                                     |         |   |
|-----------------------------------------------------|---------|---|
| KH <sub>2</sub> PO <sub>4</sub>                     | percent | 2 |
| Glycerol sorbitan laurate (G-672, Atlas Powder Co.) | percent | 6 |
| Di-2-ethylhexyl sebacate                            | Balance |   |

## Composition L

|                                                 |         |   |
|-------------------------------------------------|---------|---|
| (NH <sub>4</sub> ) <sub>2</sub> PO <sub>4</sub> | percent | 2 |
| Glycerol sorbitan laurate                       | do      | 6 |
| Mineral oil                                     | Balance |   |

Compositions of this invention were evaluated for their extreme pressure properties on a Spur Gear Machine, which consists essentially of two geometrically similar pairs of gears connected by two parallel shafts. The gear pairs are placed in separate gear boxes, which also contain the supporting ball bearings. One of the shafts consists of two sections connected by a coupling. Loading is accomplished by locking one side of the coupling and applying torque to the other. The conditions of the test were:

## TEST RESULTS

{3,000 R. P. M. pinion speed, ambient temp., 10 cc./sec. flow rate}

| Composition   | Addendum Score Load, lb. Bear Load | Tooth Face Contact | Tooth Load, lb./inch Face |
|---------------|------------------------------------|--------------------|---------------------------|
| Mineral oil   | 6                                  | Full               | 482                       |
| Composition A | 60                                 | One-half           | 8,640                     |
| Composition D | 80                                 | Full               | 5,760                     |
| Composition L | 70                                 | One-half           | 10,080                    |
| Composition E | 80                                 | Full               | 5,160                     |

Compositions of this invention were further tested in the Hypoid Gear Machine and under modified L-19-645 engine test conditions as described in the 1946 CRC Handbook published by the Coordination Research Council.

## TEST RESULTS

|                                                                                               | Hypoid Gear Machine (Chevrolet Hypoid Gears, 2,250 R. P. M. Pinion Speed) Oil Pressure (p. s. i.) | Transmitted Horse-power | Modified L-19-645 Test |
|-----------------------------------------------------------------------------------------------|---------------------------------------------------------------------------------------------------|-------------------------|------------------------|
| Mineral oil                                                                                   | 8                                                                                                 | 22                      | Failed.                |
| Mineral oil + 1% di-2-ethylhexyl amine salt of trichloromethane phosphonic acid ester mixture | 100                                                                                               | 309                     | Failed.                |
| Composition H                                                                                 | 100                                                                                               | 309                     | Passed.                |
| Composition G                                                                                 | 40                                                                                                | 124                     | Passed.                |

Compositions of this invention can be combined with other additives in lubricants, such as blooming agents, pour point depressants or viscosity improvers, antifoaming agents, e. g., dimethyl silicon polymer and the like.

5 Antioxidants comprise several types, for example, alkyl phenols such as 2,4,6-trimethyl phenol, pentamethyl phenol, 2,4-dimethyl-6-tertiary-butyl phenol, 2,4-dimethyl-6-octyl phenol, 2,6-ditertiary-butyl-4-methyl phenol, 2,4,6-tri-tertiary-butyl phenol and the like; amino phenols as benzyl amino phenols; amines such as dibutyl-phenylene diamine, diphenyl amine, N-phenyl-beta-naphthylamine, N-phenyl-alpha-naphthylamine, dinaphthyl amine.

Corrosion inhibitors or anti-rusting compounds may also be present, such as dicarboxylic acids of 16 and more carbon atoms; organic compounds containing acidic radical in close proximity to a nitrile, nitro or nitroso group (e. g., alpha-cyanostearic acid).

Wear reducing agents which may be used comprise: esters of phosphorus acids such as triaryl, alkyl hydroxy aryl, or aralkyl phosphates, thiophosphates or phosphites and the like; neutral aromatic sulfur compounds of relatively high boiling temperatures such as diaryl sulfides, diaryl disulfides, alkyl aryl disulfides, e. g., diphenyl sulfide, diphenol sulfide, dicesol sulfide, dixylenol sulfide,

25 methyl butyl diphenol sulfide, dibenzyl sulfide, corresponding di- and tri-sulfides, and the like; sulfurized fatty oils or esters of fatty acids and monohydric alcohols, e. g., sperm oil, jojoba oil, etc.; in which the sulfur is strongly bonded; sulfurized long chain olefins such as may be obtained by dehydrogenation or cracking of wax; sulfurized phosphorized fatty oils or acids, phosphorus acid esters having sulfurized organic radicals, such as esters of phosphoric or phosphorus acids with sulfurized hydroxy fatty acids; chlorinated hydrocarbons, such as chlorinated paraffin aromatic hydrocarbons, terpenes, mineral lubricating oil, etc.; or chlorinated esters of fatty acids containing the chlorine in position other than alpha position.

30 Additional ingredients may comprise oil-soluble urea or thiourea derivatives, e. g., urethanes, allophanates, carbazides, carbazones, etc.; polyisobutylene polymers, unsaturated polymerized esters of fatty acids and monohydric alcohols and other high molecular weight oil-soluble compounds.

35 Depending upon the additive used and conditions under which it is used, the amount of additive used may vary from 0.01 to 2% or higher.

40 It is to be understood that while the features of the invention have been described and illustrated in connection with certain specific examples, the invention, however, is not to be limited thereto or otherwise restricted, except by the prior art and the broad scope of the disclosed invention.

45 We claim as our invention:

1. A lubricating composition adapted for extreme pressure use comprising a major amount of mineral lubricating oil having incorporated therein from 0.1 to 10% of a salt selected from the group consisting of sodium dihydrogen phosphate, potassium dihydrogen phosphate and ammonium dihydrogen phosphate, said salt being in colloidal dimensions of from about 1 to 10 microns.

50 2. A lubricating composition adapted for extreme pressure use comprising a major amount of mineral lubricating oil having incorporated therein from 0.1 to 10% of a salt selected from the group consisting of sodium dihydrogen phosphate, potassium dihydrogen phosphate and ammonium dihydrogen phosphate in colloidal dimensions of from about 1 to 10 microns, and a minor amount sufficient to solubilize said inorganic salt of an ester of a polyhydric alcohol and a long-chain aliphatic carboxylic acid.

55 3. A lubricating composition adapted for extreme pressure use comprising a major amount of mineral lubricating oil having incorporated therein from 0.1 to 10% of a salt selected from the group consisting of sodium dihydrogen phosphate, potassium dihydrogen phosphate and

ammonium dihydrogen phosphate in colloidal dimensions of from about 1 to 10 microns, and a minor amount sufficient to solubilize said inorganic salt of glycerol sorbitan laurate.

4. A lubricating composition adapted for extreme pressure use comprising a major amount of mineral lubricating oil having incorporated therein from .01 to 10% of potassium dihydrogen phosphate in colloidal dimensions of from about 1 to 10 microns.

5. A lubricating composition adapted for extreme pressure use comprising a major amount of mineral lubricating oil having incorporated therein from .01 to 10% of ammonium dihydrogen phosphate in colloidal dimensions of from about 1 to 10 microns.

6. A lubricating composition adapted for extreme pressure use comprising a major amount of mineral lubricating oil having incorporated therein from .01 to 10% of sodium dihydrogen phosphate in colloidal dimensions of from about 1 to 10 microns.

7. A lubricating composition adapted for extreme pressure use comprising a major amount of mineral lubricating oil having incorporated therein from .01 to 10% of potassium dihydrogen phosphate in colloidal dimensions of from about 1 to 10 microns, and a minor amount sufficient to solubilize said potassium dihydrogen phosphate of glycerol sorbitan laurate.

8. A lubricating composition adapted for extreme pressure use comprising a major amount of mineral lubricating oil having incorporated therein from .01 to 10% of ammonium dihydrogen phosphate in colloidal dimensions of from about 1 to 10 microns, and a minor amount sufficient to solubilize said ammonium dihydrogen phosphate of glycerol sorbitan laurate.

9. A lubricating composition adapted for extreme pressure use comprising a major amount of mineral lubricating oil having incorporated therein from .01 to 10% of

sodium dihydrogen phosphate in colloidal dimensions of from about 1 to 10 microns, and a minor amount sufficient to solubilize said sodium dihydrogen phosphate of glycerol sorbitan laurate.

5 10. A lubricating composition adapted for extreme pressure use comprising a major amount of mineral lubricating oil having incorporated therein from .01 to 10% of potassium dihydrogen phosphate in colloidal dimensions of from about 1 to 10 microns, and from about 0.01 to about 2% of di-2-ethylhexyl amine salt of monobutyl trichloromethanephosphonic acid ester.

11. A lubricating composition adapted for extreme pressure use comprising a major amount of mineral lubricating oil having incorporated therein from .01 to 10% of ammonium dihydrogen phosphate in colloidal dimensions of from about 1 to 10 microns, and from about 0.01 to about 2% of di-2-ethylhexyl amine salt of monobutyl trichloromethanephosphonic acid ester.

12. A lubricating composition adapted for extreme pressure use comprising a major amount of mineral lubricating oil having incorporated therein from .01 to 10% of sodium dihydrogen phosphate in colloidal dimensions of from about 1 to 10 microns, and from about 0.01 to about 2% of di-2-ethylhexyl amine salt of monobutyl trichloromethanephosphonic acid ester.

#### References Cited in the file of this patent

#### UNITED STATES PATENTS

|    |           |                       |               |
|----|-----------|-----------------------|---------------|
| 30 | 2,079,051 | Sullivan et al. ----- | May 4, 1937   |
|    | 2,455,659 | Duncan et al. -----   | Dec. 7, 1948  |
|    | 2,530,837 | Orozco et al. -----   | Nov. 21, 1950 |

#### OTHER REFERENCES

35 Atlas Surface Active Agents, publication of Atlas Powder Co., Wilmington, Delaware, 1950, pages 2 and 10. (Copy in Div. 64.)